

## UNITED STATES PATENT OFFICE

2,577,110

EXPLOSIVE COMPOSITION CONTAINING  
VERMICULITE

Austin Maurice Cummings, Woodbury, N. J., assignor to E. I. du Pont de Nemours &amp; Company, Wilmington, Del., a corporation of Delaware

No Drawing. Application October 23, 1947,  
Serial No. 781,759

2 Claims. (Cl. 52—11)

1

This invention relates to an improved explosive composition of the non-nitroglycerin type in which no normally liquid component is present.

As is well known, the nitroglycerin dynamites normally include, in addition to this ingredient, one or more oxidizing agents, and combustible oxygen-acceptors such as wood pulp or various meals, these latter materials functioning also as absorbents for the nitroglycerin, so that no exudation shall take place. Explosives have been developed that are free from liquid ingredients and that are based on ammonium nitrate as the explosive ingredient, explosive or nonexplosive solid materials being present that are deficient in oxygen and that sensitize the ammonium nitrate and substantially balance it with respect to oxygen. The "Nitramon" type of explosive is a relatively recent development in such explosives, as disclosed in USP—1,992,217. This blasting agent is of a low order of sensitivity such that it is not capable of detonation by means of a commercial blasting cap but can be brought to detonation readily by a stronger booster charge. While this latter blasting agent contains ingredients that are highly susceptible to the effect of water and moisture, it is completely protected therefrom by tight enclosure within a metal container.

Cap-insensitive ammonium nitrate explosives of the type described must be controlled within predetermined close limits as to density, if satisfactory performance is to be assured. One method used for obtaining this control is by the inclusion in the composition of a relatively low density organic meal such as a comminuted flaked corn product or its substantial equivalent. Such organic materials have not been satisfactory, however, inasmuch as they increase the combustibility of the product and thus affect the safety properties adversely, especially when elevated temperatures may be employed during manufacture and incorporation.

An object of the present invention is an improved explosive composition of the non-nitroglycerin type, in which ammonium nitrate is the principal explosive ingredient. A further object is such a composition of a low order of sensitivity to detonation and of a relatively high density. A still further object is such an ammonium nitrate composition in which a low density ingredient is included that facilitates satisfactory density control but has no unfavorable effect on the flammability and safety properties. Additional objects will be disclosed as the

invention is described at greater length herein-after.

I have found that the foregoing objects are accomplished, and a highly desirable product obtained, when I employ an explosive composition free from normally liquid ingredients, explosive or non-explosive, and comprising at least one inorganic oxidizing agent, at least one organic combustible ingredient functioning as an oxygen-acceptor and as a sensitizer for the oxidizing agent, and a relatively small proportion of a low density, expanded hydrated silicate. The inorganic oxidizing agent will preferably be ammonium nitrate because of its known properties and its ability to enter into explosive reactions effectively. Various organic sensitizers may be employed such as paraffin, nitrotoluene, coal, and the like. As the low density silicate, we find the mineral vermiculite particularly desirable in its expanded or exfoliated form, as a result of treatment at high temperatures.

The following composition illustrates one embodiment of an ammonium nitrate explosive formula in accordance with the disclosures of the present invention. It will be understood that the composition given is by way of example only and is not to be taken as limiting in any way.

|                        | Percent |
|------------------------|---------|
| Ammonium nitrate       | 61.0    |
| Sodium nitrate         | 23.0    |
| Paraffin               | 4.0     |
| Dinitrotoluene         | 8.0     |
| Vermiculite (expanded) | 4.0     |
|                        | 100.0   |

In preparing the above mixture, ammonium nitrate of the predetermined degree of fineness was blended with the sodium nitrate and heated to 54° C., and paraffin was then added and mixed for 10 minutes. Dinitrotoluene was added and mixed for an additional 10 minutes, then the vermiculite, with additional 5 minute mixing. The finished mixture was discharged at a temperature of around 63° C. At a density of 1.00, the composition was insensitive to the action of seven No. 8 blasting caps. When packed into tightly sealed cans, 4 in. x 24 in. in dimensions, and primed with a suitable TNT booster, the explosion was propagated from one can to another with an undiminished velocity of detonation of around 3400 meters per second. To illustrate the improvement with respect to flammability by the replacement of organic low density combustibles by the expanded vermiculite, the following results are conclusive on compar-

ble formulas containing different low density ingredients:

| Low Density Ingredient | Ignition Time at 136° C. |
|------------------------|--------------------------|
|                        | Hours                    |
| Skinned Corn Product   | 7½                       |
| Gassee Pith            | 8½                       |
| Expanded Vermiculite   | 24                       |

The present invention is applicable to various types of explosive compositions that are free from liquid ingredients, whether liquid explosives such as nitroglycerin or non-explosive liquids. Absorptive properties in the case of this low density ingredient are not under consideration, therefore, as they would be for such materials in nitroglycerine dynamites. While ammonium nitrate explosives are the compositions in which the ingredient has been found particularly advantageous, its use is not limited to such mixtures but is applicable in compositions based on other suitable inorganic oxidizing agents, for example ammonium perchlorate, potassium perchlorate, sodium nitrate, blends of sodium and ammonium nitrate, etc. As has been noted, particular advantage is found in its inclusion in sensitized ammonium nitrate blasting agents of a low degree of sensitivity, such that they cannot be detonated by one or more commercial blasting caps. Such compositions are ordinarily packed into watertight containers at high density, for example above 1.0. It is important with such compositions to control the density closely, in order that they shall remain sufficiently sensitive to propagate the explosion when this has been once initiated and that at the same time they shall not lose their superior safety properties and become detonable by relatively weak primers.

The inclusion of an organic low density material, such as a meal or flour, is definite in its effect on the density of the explosive composition but, as already pointed out, introduces someammability hazards. Such low density ingredient is ordinarily in finely divided form and as such as is quite reactive with inorganic oxidizing agents. While such blends are stable at ordinary temperatures, more elevated temperatures are often experienced during manufacture and handling. In the case of ammonium nitrate compositions that are packed in metal cans, for example, the sealing of the open end of the can after loading requires high temperatures, as in the soldering operation. When organic meals are used, local burning of the charge is a definite hazard.

The use of the inorganic expanded hydrated silicate in relatively finely divided form, in accordance with the present invention, not only gives all the advantages of density control obtained by the employment of organic meals but at the same time introduces no safety hazards; in fact, its presence improves the safety properties. The material particularly favored for such use comprises the mineral vermiculite which has been expanded by subjection to high temperatures. Vermiculite is an alteration prod-

uct of mica and in composition is a complex hydrated aluminum-iron-magnesium silicate. It possesses the unusual property of exfoliating or expanding when heated to high temperatures, due to the fact that it normally is made up of extraordinarily large numbers of layers per inch with a very small amount of water between each layer. When subjected to high temperatures, the water becomes converted to steam, whereby the flakes expand into cellular grains of many times their original size. During this expansion, a great number of closed air cells are formed and the entrapped air insures its permanent low density. Other, normally anhydrous silicious materials, kieselguhr for example, do not possess this property, and do not function in the manner described for expanded vermiculite. The material as used will desirably have an apparent density of around 0.16 gram per cc. or less and a degree of fineness such that it will all pass a 6-mesh and be largely held on a 14-mesh screen. The water content should be low.

While various explosive compositions embodying the ingredients mentioned are suitable, we find a desirable mixture to comprise more than 50% ammonium nitrate, between 0.5 and 10.0% of a normally solid paraffin hydrocarbon, between 0.5 and 10.0% of an aromatic nitrocompound, and between 1.0 and 8.0% of vermiculite in expanded form. Dinitrotoluene will be a satisfactory aromatic nitrocompound, or a blend of nitrotoluenes.

The invention has been described at length in the foregoing. It will be understood, however, that many variations may be introduced in compositions used, procedures followed, or types of explosive compositions, without departure from the scope of the invention.

I intend to be limited, therefore, only by the following claims.

I claim:

1. A high velocity detonating explosive containing only normally solid ingredients and comprising ammonium nitrate in an amount, greater than 50% of the composition, at least one normally solid organic sensitizing agent for the ammonium nitrate, and between 1.0 and 8.0% of vermiculite in expanded form.

2. A high velocity detonating explosive comprising more than 50% ammonium nitrate, between 0.5 and 10.0% of a normally solid paraffin hydrocarbon, between 0.5 and 10.0% of a normally solid aromatic nitrocompound, and between 1.0 and 8.0% of vermiculite in expanded form.

AUSTIN MAURICE CUMMINGS.

#### REFERENCES CITED

The following references are of record in the file of this patent:

#### UNITED STATES PATENTS

| Number    | Name       | Date          |
|-----------|------------|---------------|
| 1,743,744 | Winkelmann | Jan. 14, 1930 |
| 1,881,307 | Bashford   | Oct. 4, 1932  |
| 1,964,222 | Scott      | June 26, 1934 |
| 1,992,217 | Kirst      | Feb. 26, 1935 |
| 2,463,927 | Watts      | Mar. 8, 1949  |